

Nov. 14, 1961

J. R. SIEGEL

3,008,813

HYDROCARBON OILS HAVING IMPROVED WATER TOLERANCE

Filed Oct. 29, 1958

EFFECT OF DICOCO DIMETHYL AMMONIUM CHLORIDE  
UPON HAZE SETTLING RATE



Joel R. Siegel

Inventor

By *James E. Reel*

Attorney

## 1

3,008,813

HYDROCARBON OILS HAVING IMPROVED  
WATER TOLERANCE

Joel R. Siegel, Irvington, N.J., assignor to Esso Research  
and Engineering Company, a corporation of Delaware  
Filed Oct. 29, 1958, Ser. No. 770,520  
12 Claims. (Cl. 44—62)

The present invention relates to improvements in the water tolerance of hydrocarbon oils and more particularly relates to petroleum distillate fuels and similar hydrocarbon oil products having incorporated therein additive agents singularly adapted to prevent the formation of persistent haze and stable emulsions when such products are contacted with water during handling and storage.

Ashless oil-soluble polymeric dispersants have largely displaced metal sulfonates, metal naphthenates and similar compounds for use as stabilizing additives in petroleum distillate fuels and related hydrocarbon oil products because of their increased ability to suspend insoluble degradation products formed in such oils. Sludge and sediment which might otherwise tend to clog fuel lines, orifices, screens and filters through which the oils must pass are held in suspension to a much greater extent by the polymeric additives than by the additive materials formerly employed. These increased dispersive properties, although highly desirable from the standpoint of oil stability, have given rise to water tolerance problems much more serious than those heretofore encountered. The polymeric materials employed as oil stabilizing additives exhibited particularly pronounced tendencies to suspend any water with which the oils come into contact and hence extremely persistent haze and stable emulsions are formed upon contact of oils containing the polymeric additives with water. Since an aqueous phase exists in most tanks and other vessels containing such oils, haze formation and emulsification are almost impossible to avoid. As a consequence, the marketability of distillate fuels, lubricating oils, transformer oils, turbine oils and other petroleum distillate products in which polymeric dispersants are used is often seriously affected.

The present invention provides a class of new and improved additives which are surprisingly effective for increasing the water tolerance of petroleum distillate fuels and similar liquid hydrocarbon oils containing polymeric dispersant additives. In accordance with the invention, it has now been discovered that the addition of minor amounts of certain quaternary ammonium compounds to such oils greatly reduces the persistence of haze and emulsions formed when the products are contacted with water and thus permits their transportation and storage in the presence of an aqueous phase without adverse results.

The quaternary ammonium compounds which have been found to be singularly effective for improving the water tolerance of petroleum products in accordance with the invention are dialkyl dimethyl ammonium chlorides having alkyl groups which each contain from 12 to 14 carbon atoms. It has been found that compounds of this type are critical for purposes of the invention. Closely related tetraalkyl ammonium chlorides such as the trialkyl monomethyl ammonium chlorides and the monoalkyl trimethyl ammonium chloride are not effective for reducing haze and emulsion formation, are readily extracted by water, adversely affect the action of the polymeric stabilizing additives, or are otherwise unsuitable for purposes of the invention. Specific examples of dialkyl dimethyl ammonium chlorides which may be employed are didodecyl dimethyl ammonium chloride, ditridecyl dimethyl ammonium chloride, dodecyl tridecyl dimethyl ammonium chloride, dodecyl tetradecyl dimethyl ammonium chloride and tridecyl tetradecyl dimethyl am-

## 2

monium chloride. Also useful for purposes of the invention are dialkyl dimethyl ammonium chlorides derived from naturally occurring materials such as coconut oil which contain at least 50% by weight of  $C_{12}$  to  $C_{14}$  alkyl groups. Dicocodimethyl ammonium chloride, derived from coconut oil, contains from about 55 to about 70% of  $C_{12}$  to  $C_{14}$  alkyl groups and has been found eminently satisfactory for purposes of the invention. The alkyl groups outside the  $C_{12}$  to  $C_{14}$  range in these mixed dialkyl dimethyl ammonium chlorides apparently do not contribute to the improved water tolerance of the products to which the chlorides are added but appear to have no adverse effect. Such mixed dialkyl dimethyl ammonium chlorides are generally referred to as technical dilauryl dimethyl ammonium chlorides and are readily available from commercial sources. Such mixtures are therefore preferred for purposes of the invention.

The polymeric dispersant additives primarily responsible for the poor water tolerance of distillate fuels and similar products are widely used commercially and are well known to those skilled in the art. These dispersants in general are polymers and copolymers of unsaturated organic esters, nitriles and similar monomers containing vinyl, vinylene or vinylidene linkages. The dialkyl dimethyl ammonium chlorides employed in accordance with the invention have been found effective when used in oils containing a wide variety of such polymeric dispersants.

A class of polymeric dispersant additives in conjunction with which the dialkyl dimethyl ammonium chlorides have been found to be particularly effective are those which are prepared by the copolymerization of an alkyl chloropropyleneoxy mixed ester of an unsaturated conjugated dibasic acid with a polymerizable organic monomer containing a vinyl linkage. The alkyl chloropropyleneoxy mixed esters used as one of the components of such copolymers are prepared by first reacting a  $C_4$  to  $C_5$  unsaturated conjugated dibasic acid such as maleic acid, fumaric acid, citraconic acid, mesaconic acid or a mixture of such acids or their anhydrides, when they exist, with a long chain saturated aliphatic alcohol to produce a half ester. Suitable alcohols for this purpose are those containing from about 8 to about 24 carbon atoms per molecule, preferably about 8 to 18 carbon atoms per molecule. Straight chain primary alcohols such as dodecyl, cetyl, eicosyl and docosyl alcohols are preferred but branched chain alcohols such as 2-ethylhexanol-1 and  $C_8$  oxo-alcohols, secondary alcohols such as capryl alcohol and mixtures of straight and branched-chain alcohols may also be used. Commercially marketed mixtures of alcohols of the requisite chain length, such as those obtained by the hydrogenation of coconut oil may also be used.

The half ester produced in the above manner is then reacted with epichlorohydrin in the presence of either an acidic or a basic catalyst such as boron fluoride or sodium hydroxide to produce the mixed ester. The ratio of the half ester to epichlorohydrin in the reaction mixture may range from about 1:1 to 1:4. Addition of the epichlorohydrin takes place through the epoxy group and the chlorine atom is unaffected. The mixed ester may thus contain from 1 to about 3 chlorine atoms.

The mixed ester prepared as described above is then copolymerized with from about  $\frac{1}{2}$  to about 20 parts of an unsaturated organic monomer containing a vinyl group in the presence of gamma radiation, a peroxide type catalyst such as benzoyl peroxide, or an azo catalyst such as alpha-alpha azo-bis-isobutyronitrile. Suitable monomers containing vinyl groups include hydrocarbons such as styrene, isobutylene and butadiene; esters such as vinyl propionate and methyl methacrylate; ethers such as di-vinyl ether; and nitriles such as acrylonitrile and vinyl-acetonitrile. Mixtures of such monomers containing

vinyl groups with other copolymerizable materials, long chain alcohol esters of unsaturated conjugated dibasic acids such as lauryl maleate and tallow fumarate for example, may also be used. Vinyl esters of short chain fatty acids, particularly vinyl acetate and mixtures of such esters with fumarate or maleate esters of long chain aliphatic alcohols containing from about 8 to about 20 carbon atoms per molecule are preferred monomers for preparation of the copolymers with the mixed esters.

The resulting copolymers are oil-soluble and preferably have molecular weights between about 6000 and about 20,000 Staudinger. Such copolymers are described in copending application S.N. 673,156, filed July 22, 1957.

A second class of polymeric dispersant additives with which the dialkyl dimethyl ammonium chlorides are especially effective are oil-soluble, nitrogen-containing addition type copolymers prepared by copolymerizing an amine-free monomer containing one polymerizable ethylenic linkage and an aliphatic hydrocarbon chain of from 8 to 18 carbon atoms with a monomer containing a nitrogen atom and one polymerizable ethylenic linkage. Such copolymers may be prepared, for example, by the copolymerization of an acrylic or alpha-substituted acrylic ester of an aliphatic alcohol containing an average of from 8 to 18 carbon atoms, such as lauryl methacrylate, with an ethylenically unsaturated compound containing a basic amino group, such as beta dimethylamino-ethyl methacrylate. Other specific examples of the amine-free monomers containing a polymerizable ethylenic linkage and a C<sub>8</sub>-C<sub>18</sub> aliphatic chain include the tridecyl, cetyl and octadecyl esters of acrylic and methacrylic acids. Also suitable are esters of these acids prepared from mixtures of alcohols such as those containing primary alcohols of from 10 to 18 carbon atoms derived by the hydrogenation of coconut oil and sold under the trade name "Lorol." A typical mixture consists chiefly of lauryl alcohol having 12 carbon atoms per molecule and has the following approximate composition:

| Alcohol constituent—               | Weight percent |
|------------------------------------|----------------|
| C <sub>10</sub> H <sub>21</sub> OH | 4.0            |
| C <sub>12</sub> H <sub>25</sub> OH | 55.5           |
| C <sub>14</sub> H <sub>29</sub> OH | 22.5           |
| C <sub>16</sub> H <sub>33</sub> OH | 14.0           |
| C <sub>18</sub> H <sub>37</sub> OH | 4.0            |

The polymerizable ethylenically unsaturated compounds containing a nitrogen-containing group which are used in forming the second class of preferred copolymers suitable for use in accordance with the invention include the basic tertiary amino-alkyl acrylates, such as the dialkyl amino-alkyl acrylates and alpha hydrocarbon-substituted acrylates, beta dimethylaminoethyl acrylate and methacrylate, and their homologs and analogs. The nitrogen may be a member of a heterocycle where the polymerizable ethylenic unsaturation is extra-nuclearly bonded to the heterocycle, such as the vinyl pyridines and vinyl pyrrolidone.

Limited amounts of other copolymerizable monomers in addition to those described above may be incorporated into the copolymers of the second preferred class as filler materials. Such filler materials include vinyl and allyl formates, acetates, propionates; isobutylene; styrene; methyl methacrylate; ethyl vinyl ether and the like. The final copolymer may contain from about 20% to about 99% of the nitrogen-free monomer, from about 0.5% to 50% of the nitrogen-containing monomer, and from about 0 to about 79% of the monomer used as a filler material. Many of the polymeric additives falling within the second preferred class described above are described in detail in U.S. Patent No. 2,737,452, issued March 6, 1956.

Polymeric dispersant additives of the second class described above are sometimes employed in combination with tertiary alkyl primary amines. Although such amines do not have pronounced dispersant properties,

they effect a considerable improvement in the stabilizing action of the nitrogen-containing polymeric dispersants. They do not, however, overcome the tendency of such dispersants to suspend water in oils in which they are present and hence do not prevent the water tolerance problem caused by the dispersants. The dialkyl dimethyl ammonium chlorides may therefore be employed to advantage in oils containing both a polymeric dispersant and a tertiary alkyl primary amine.

The tertiary alkyl primary amines useful with the polymeric dispersants described above in general are those having two alkyl groups of from 1 to 3 carbon atoms attached to the tertiary carbon atom and one alkyl group of from 5 to 21 carbon atoms attached to the tertiary carbon atom. Tertiary alkyl primary amines containing a total of from 8 to 18 carbon atoms per molecule are preferred. Particularly preferred are C<sub>12</sub> tertiary alkyl primary amines. Mixtures of such amines such as those derived from polyolefins may also be used.

Tertiary alkyl primary amines such as those described above are generally employed in combination with the nitrogen-containing polymeric dispersants in concentrations such that the ratio of amine to dispersant in the oil ranges from about 2 to 1 to about 18 to 1. Amine concentrations between about 0.003 wt. percent to about 0.8 wt. percent are especially effective.

Many other polymeric dispersant additives suitable for the stabilization of hydrocarbon oils will be familiar to those skilled in the art. The stabilization of haze and emulsions is a universal property of such dispersant additives and the dialkyl dimethyl ammonium chlorides may be employed with a wide variety of such materials. Representative examples of other ashless, oil-soluble polymeric stabilizing additives are described in U.S. Patent 2,737,496 to Catlin; in U.S. 2,800,452 to Bondi et al.; and in application S.N. 690,184, filed October 15, 1957, now U.S. Patent 2,958,590.

The oils in which the additives of the invention may be incorporated are liquid petroleum distillate products boiling in the range between about 75° and about 900° F. Such products include gasolines, aviation turbo-jet fuels, kerosenes, diesel fuels, transformer oils, turbine oils, heating oils, and lubricating oils. The additives are particularly effective in distillate fuels boiling in the range between about 250° F. and about 750° F. Such fuels include turbo-jet engine fuels, diesel fuels and heating oils which have particularly poor stability properties and require the use of relatively large amounts of the polymeric dispersant additives. Aviation turbo-jet engine fuels are defined by U.S. Military Specifications MIL-F-5624C, MIL-F-25524A, and MIL-F-2258A and are generally referred to as JP-4, JP-5 and JP-6. Diesel fuels in connection with which the additives of the invention are particularly useful are more fully described in ASTM Specification D-975-53T and may be used in stationary, marine and automotive type engines. Typical of the heating oils in which the additives may be employed are those described in ASTM Specification D-396-48T, particularly those in grades 1 and 2 there-

of.

The polymeric dispersant additives are generally employed in petroleum hydrocarbon products such as those described above in concentrations ranging from about 0.001% and about 1% by weight. Concentrations of from 0.001% to 0.05% are generally preferred. The dialkyl dimethyl ammonium chlorides which are used in such oils may be incorporated therein in concentrations in the range of from about 0.00025 wt. percent to about 0.01 wt. percent. Chloride concentrations in the range of from about 0.0005 wt. percent to about 0.001 wt. percent have been found to be generally effective and are preferred, since it has been found that the stabilizing properties of some dispersant additives may suffer when the dialkyl dimethyl ammonium chlorides are present in very high concentrations.

The ammonium chloride compound may be incorporated into the fuels by dissolving them in a suitable solvent such as isopropanol, butanol, benzene or the like and then adding the resultant solution to the oil in quantities sufficient to give the desired additive concentrations. If desired, additive concentrates containing both the polymeric dispersant stabilizing additive and the dialkyl dimethyl ammonium chloride compound in a suitable solvent may be prepared. Other additive materials commonly used in the products to which the concentrate is to be added may also be included in such concentrates. Such other additive materials may comprise rust inhibitors, anti-static additives, corrosion inhibitors, dyes, dye stabilizers and the like.

The invention may be further illustrated by the following examples and the accompanying drawing.

#### EXAMPLE 1

Samples of a petroleum distillate heating oil which had been stabilized by the inclusion therein of 0.01% by weight of various polymeric dispersant additives were tested to determine the persistence of the haze formed when the fuel was contacted with water and the stability of the emulsions formed during such contacting. The fuel employed was a blend consisting of about 50% by volume of virgin gas oil and about 50% by volume of catalytically cracked stock. Typical inspections for a fuel of this type are as follows:

|                                       |       |
|---------------------------------------|-------|
| Gravity, ° API                        | 34.6  |
| Color, Tag-Robinson                   | 16½   |
| Pensky-Martens flash, ° F             | 185   |
| Sulfur, wt. percent                   | 0.32  |
| Neutralization No                     | 0.02  |
| Aniline point, ° F                    | 109.5 |
| ASTM distillation:                    |       |
| Initial boiling point, ° F            | 324   |
| 10% point, ° F                        | 396   |
| 50% point, ° F                        | 482   |
| 90% point, ° F                        | 597   |
| Final boiling point, ° F              | 643   |
| Conradson carbon residue, wt. percent | 0.006 |

The persistence of the haze formed in this oil upon contact with water was measured in Waring Blender haze tests wherein five milliliters of water and 500 milliliters of the oil were mixed in a Waring Blender for a period of five minutes, the oil-water mixture was then allowed to stand for six hours, and the amount of light which was transmitted through the oil under standardized conditions was measured. The light transmission was expressed as a percentage of the total light emitted from the source. This test has been found to be an extremely effective means for determining the degree to which haze is present in hydrocarbon oils and is recognized as reliable throughout the petroleum industry.

Herschel emulsion tests were carried out to determine the effect of the additives upon emulsification by stirring 40 milliliters of oil and 40 milliliters of water for five minutes at a temperature of 77° F. to form an emulsion, letting the mixture stand for 15 minutes, and then measuring the volume of the emulsion phase. Similar tests are widely used for determining the emulsification tendencies of turbine oils in accordance with ASTM Standard D-1401-56T and in similar applications.

Three different tetraalkyl ammonium chlorides were added in concentrations of 0.0008 wt. percent to separate samples of the same heating oil containing 0.01 wt. percent of the same polymeric dispersant additive. The tetraalkyl ammonium chlorides employed were as follows:

(1) Dicoco dimethyl ammonium chloride—a dialkyl dimethyl ammonium chloride having mixed alkyl groups derived from coconut oil as follows: 8% C<sub>8</sub> radicals, 7% C<sub>10</sub> radicals, 48% C<sub>12</sub> radicals, 18.5% C<sub>14</sub> radicals, 8% C<sub>16</sub> radicals and 10.5% C<sub>18</sub> radicals.

(2) Disoya dimethyl ammonium chloride—a dialkyl

dimethyl ammonium chloride having mixed alkyl groups derived from soybean oil which include about 8% C<sub>16</sub> radicals, about 88% C<sub>18</sub> radicals and about 4% C<sub>20</sub> radicals.

(3) Dihydrogenated tallow dimethyl ammonium chloride—a dialkyl dimethyl ammonium chloride having mixed C<sub>16</sub> and C<sub>18</sub> alkyl groups derived from hydrogenated tallow.

(4) Tallow trimethyl ammonium chloride—a monoalkyl trimethyl ammonium chloride having mixed C<sub>16</sub> and C<sub>18</sub> alkyl groups derived from tallow.

The oil samples containing the polymeric dispersant additive and the above tetraalkyl ammonium chlorides were then subjected to Waring Blender haze tests and Herschel emulsion tests, both with and without prior water extraction. About 1% water was used in the water extraction step. The results obtained in these tests are in Table I.

Table I

#### EFFECT OF TETRAALKYL AMMONIUM CHLORIDES UPON HAZE AND EMULSIFICATION IN HEATING OILS

| Fuel                                                                                      | Waring Blender haze test, percent light transmission after 6 hours |                           | Herschel emulsion test, milliliters emulsion after 15 minutes |                           |
|-------------------------------------------------------------------------------------------|--------------------------------------------------------------------|---------------------------|---------------------------------------------------------------|---------------------------|
|                                                                                           | Fuel not water extracted                                           | Fuel extracted with water | Fuel not water extracted                                      | Fuel extracted with water |
| Base heating oil                                                                          | 94                                                                 | -----                     | 0                                                             | 0                         |
| Base heating oil+0.01% additive A <sup>1</sup>                                            | 14                                                                 | 12                        | 4                                                             | 31                        |
| Base heating oil+0.01% additive A+0.008% dicoco dimethyl ammonium chloride                | 95                                                                 | 81                        | 1                                                             | 2                         |
| Base heating oil+0.01% additive A+0.008% disoya dimethyl ammonium chloride                | 54                                                                 | 30                        | 3                                                             | 18                        |
| Base heating oil+0.01% additive A+0.008% dihydrogenated tallow dimethyl ammonium chloride | 53                                                                 | 12                        | 18                                                            | 15                        |
| Base heating oil+0.01% additive A+0.008% tallow trimethyl ammonium chloride               | 90                                                                 | 6                         | -----                                                         | -----                     |
| Base heating oil+0.01% additive B <sup>2</sup>                                            | 48                                                                 | 64                        | -----                                                         | -----                     |
| Base heating oil+0.01% additive B+0.008% dicoco dimethyl ammonium chloride                | 92                                                                 | 88                        | -----                                                         | -----                     |
| Base heating oil+0.01% additive B+0.008% disoya dimethyl ammonium chloride                | 36                                                                 | 60                        | -----                                                         | -----                     |
| Base heating oil+0.01% additive B+0.008% dihydrogenated tallow dimethyl ammonium chloride | 29                                                                 | 27                        | -----                                                         | -----                     |

<sup>1</sup> Additive A was a copolymer of 1 mol of vinyl acetate, 0.25 mol of isooctyl chloropropyleneoxy maleate, and 0.75 mol of mixed C<sub>16</sub>-C<sub>18</sub> alkyl fumarates, 50 weight percent concentration in benzene.

<sup>2</sup> Additive B was a mixture of 8 parts of a C<sub>12</sub> tertiary alkyl primary amine and 1 part of a copolymer prepared from 8 parts of Lorol methacrylate and 2 parts of beta diethylaminoethyl methacrylate.

From the Waring Blender test results in the above table it can be seen that the light transmission through the base heating oil containing the polymeric dispersant additive was quite low, indicating a high haze level. The fact that this haze persisted even though six hours had elapsed between the time the water and oil were mixed and the time the light transmission values were determined shows that it was exceptionally stable due to the presence of the polymeric dispersant in the oil. The results obtained with the samples containing the dicoco dimethyl ammonium chloride demonstrate the remarkable effectiveness of this additive for preventing the formation of persistent haze in oils. This effectiveness is particularly outstanding in view of the fact that this material is marketed commercially for use as a general emulsion stabilizer and might therefore be expected to promote,

rather than hinder, the formation of persistent haze. The disoja dimethyl ammonium chloride and the dihydrogenated tallow ammonium chloride, both of which have structures very similar to that of dicoco dimethyl ammonium chloride but do not contain predominantly  $C_{12}$  and  $C_{14}$  alkyl groups, were much less effective. Results of the Herschel emulsion tests confirm these findings. The above data also demonstrate that the effectiveness of dicoco dimethyl ammonium chloride is not seriously affected by water extraction. The disoja dimethyl ammonium chloride and the dihydrogenated tallow ammonium chloride, on the other hand, were much less effective after water extraction.

The data obtained with tallow trimethyl ammonium chloride demonstrate that a satisfactory additive must not be extracted by water to any significant extent. The tallow trimethyl ammonium chloride was largely removed from the fuel during the extraction step and hence afforded little protection against the formation of persistent haze when the fuel was subsequently subjected to the Waring Blender test. The dicoco dimethyl ammonium chloride, on the other hand, was extracted only to a slight degree and was nearly as effective following the water extraction step as it was prior to water extraction. Since distillate fuels and other petroleum products in which polymeric dispersant additives are frequently employed are often contacted with relatively large quantities of water under conditions which may lead to the extraction of additives contained therein, this difference between the dicoco dimethyl ammonium chloride and the tallow trimethyl ammonium chloride is a significant one.

#### EXAMPLE 2

In order to determine the effectiveness of commercial demulsifiers for use in oils containing polymeric dispersant additives, tests similar to those described above were carried out upon samples of heating oils containing such inhibitors. The heating oils employed had properties similar to those of the oil used in the preceding example and contained polymeric dispersants in 0.01 wt. percent concentrations. The samples were first subjected to Waring Blender haze tests. If the results from this test indicated that the particular inhibitor showed promise, Herschel emulsion tests were carried out. The overall results obtained are summarized as follows.

the haze cleared. Sixty-three of these commercial additives were found to promote haze in the presence of the polymeric dispersant, six had no visible influence upon the hazing properties of the oil containing the dispersant, and one indicated a slight improvement in haze clearing rate. When this latter additive was retested, the results could not be duplicated.

#### EXAMPLE 3

Tests were carried out to determine the effect of dicoco dimethyl ammonium chloride upon the stability of distillate petroleum products. The test employed was the accelerated storage stability test described in detail in "New Fast Test Method for Distillate Storage Stability," by W. A. Konrad, N. L. Shipley and T. S. Tutwiler on page 145 of "Petroleum Processing" for September 1946. Briefly, the accelerated filter plugging test consists of heating a sample of the oil to be tested at a controlled rate for 16 hours to a final temperature of 230° F. in order to accelerate the formation of sediment in the oil. The oil sample is then cooled and passed through a felt filter pad at a constant rate of 1 gallon per hour. As sediment accumulates on the filter under constant oil flow conditions, the pressure drop across the filter increases. After 12 liters, the Standard Volume used in the test, has been filtered, a record is made of final pressure drop across the filter, the weight of sediment collected is determined, and the appearance of the filter is noted. These criteria are individually interpreted on a demerit basis wherein 0 is an excellent rating and 10 is a very bad rating. The values for the 3 criteria, final pressure drop, weight of sediment and appearance, are averaged arithmetically to obtain the overall accelerated filter plugging test demerit value for the oil. Results obtained in this test are reproducible to  $\pm 0.3$ .

The oil employed in the accelerated filter plugging tests was a heating oil having properties substantially the same as those of the oil described in Example 1. Tests were also made on samples of this oil containing the polymeric dispersant additives described in Examples 1 and 2 and upon samples containing both the polymeric dispersant additives and dicoco dimethyl ammonium chloride. The results of these tests are set forth in Table III.

Table III

EFFECT OF DICOCO DIMETHYL AMMONIUM CHLORIDE ON FUEL STABILITY

| Inhibitor                | Dispersant additive | Waring Blender haze test, percent light transmitted after 6 hours | Herschel emulsion test, milliliters emulsion after 15 minutes | Fuel | Accelerated filter plugging test overall demerit |
|--------------------------|---------------------|-------------------------------------------------------------------|---------------------------------------------------------------|------|--------------------------------------------------|
| None                     | A <sup>1</sup>      | 3                                                                 | 5                                                             | 50   | 9.3                                              |
| Nalquat G-8-11 (0.001%)  | A                   | 3                                                                 | 5                                                             | 55   | 1.0                                              |
| Nalquat G-8-12 (0.001%)  | A                   | 3                                                                 | 5                                                             |      | 0.7                                              |
| Nalquat G-8-13 (0.001%)  | A                   | 61                                                                | 12                                                            |      |                                                  |
| Nalquat G-8-13 (0.0008%) | A                   | 3                                                                 | 5                                                             | 60   | 1.3                                              |
| Nalquat G-9-12 (0.001%)  | A                   | 43                                                                | 4                                                             |      | 1.0                                              |
| Nalquat G-9-13 (0.001%)  | A                   | 64                                                                | 5                                                             |      |                                                  |
| Nalquat G-9-13 (0.0008%) | A                   | 4                                                                 | 5                                                             |      |                                                  |
| None                     | None                | 94                                                                | 5                                                             |      |                                                  |
| Do                       | B <sup>2</sup>      | 58                                                                | 5                                                             |      |                                                  |
| Tretolite F-46 (0.01%)   | B                   | 25                                                                | 5                                                             |      |                                                  |
| Tretolite F-65 (0.01%)   | B                   | 15                                                                | 5                                                             |      |                                                  |
| Tretolite F-66 (0.01%)   | B                   | 8                                                                 | 5                                                             |      |                                                  |
| Tretolite F-66 (0.01%)   | B                   | 32                                                                | 5                                                             |      |                                                  |
| Tretolite F-45 (0.01%)   | B                   | 28                                                                | 5                                                             |      |                                                  |
| Tretolite F-97 (0.01%)   | B                   | 33                                                                | 5                                                             |      |                                                  |
| Tretolite F-98 (0.01%)   | B                   | 33                                                                | 5                                                             |      |                                                  |
| Tretolite F-90 (0.01%)   | B                   | 15                                                                | 5                                                             |      |                                                  |

NOTE.—For footnotes 1 and 2 see Table I.

Tests were carried out on 70 other commercial demulsifiers by adding 0.005 wt. percent of the material to be tested to 250 ml. of heating oil containing 0.01 wt. percent of polymeric dispersant B, shaking the sample with 1% water, and then usually observing rate at which

From the foregoing table it is evident that the addition of dicoco dimethyl ammonium chloride to petroleum distillate fuels and products containing polymeric dispersant additives does not adversely effect the stability of such fuels or interfere with the stabilizing action of the polymeric additives. At the concentrations in which they are used, the ammonium chloride compounds reduce the ability of the dispersants to suspend water but do not reduce their ability to suspend insoluble reaction products formed in the oil. The data in Table III sug-

gest that in some instances it may be preferred to limit the amount of dicoco dimethyl ammonium chloride added to oils containing polymeric dispersant stabilizing additives to about 0.001 wt. percent or less. The demerit rating of the sample containing 0.01% of dispersant A and 0.0005% of the chloride was slightly better than that of the sample containing the same amount of the polymeric dispersant and 0.001% of the chloride. The data are consistent within the reproducibility of the test.

#### EXAMPLE 4

Further tests similar to those described in the preceding examples were carried out in order to demonstrate the effect of the additives of the invention upon fuels and similar hydrocarbon oils employed in contact with aqueous pipeline corrosion inhibitor. Samples of a base heating oil containing 0.01 wt. percent of a commercial polymeric dispersant additive and various amounts of dicoco dimethyl ammonium chloride were extracted with 0.1 vol. percent of a commercial pipeline inhibitor solution. These extracted samples were then subjected to Waring Blender haze tests. The results of these tests are shown in Table IV.

Table IV

#### EFFECT OF EXTRACTION WITH PIPELINE INHIBITOR UPON TETRAALKYL AMMONIUM CHLORIDE HAZE PREVENTIVE

| Fuel                                                                                            | Percent light transmission after 6 hrs. following extraction with pipeline inhibitor solution <sup>1</sup> |
|-------------------------------------------------------------------------------------------------|------------------------------------------------------------------------------------------------------------|
| Base fuel+0.01% polymeric dispersant B <sup>2</sup>                                             | 51                                                                                                         |
| Base fuel+0.01% polymeric dispersant B <sup>2</sup> +0.00076% dicoco dimethyl ammonium chloride | 94                                                                                                         |
| Base fuel+0.01% polymeric dispersant B <sup>2</sup> +0.00068% dicoco dimethyl ammonium chloride | 90                                                                                                         |
| Base fuel+0.01% polymeric dispersant B <sup>2</sup> +0.00060% dicoco dimethyl ammonium chloride | 84                                                                                                         |
| Base fuel+0.01% polymeric dispersant B <sup>2</sup> +0.0005% dicoco dimethyl ammonium chloride  | 96                                                                                                         |

<sup>1</sup> The inhibitor was an aqueous solution used commercially for preventing pipeline corrosion and consists of 720 gms. of NaNO<sub>2</sub> and 8.6 gms. of NaOH in 2,000 ml. of distilled water.

<sup>2</sup> See footnote 2, Table III.

The above data demonstrate that the aqueous pipeline inhibitor solution did not extract the dicoco dimethyl ammonium chloride from the fuel to an appreciable extent and hence did not increase the tendency of the fuel to form persistent haze when subsequently contacted with water. The results shown above also show the effect of varying the concentration of the dicoco dimethyl ammonium chloride and indicate that the additive is particularly effective at concentrations of about 0.0005 wt. percent.

#### EXAMPLE 5

It has been found that the dialkyl dimethyl ammonium chlorides employed in accordance with the invention are effective for preventing the formation of persistent haze in hydrocarbon oils only in cases where the chlorides are present in the oil prior to its being contacted with water. The additive does not resolve haze which is already present in the oil. This is illustrated by a series of tests wherein dicoco dimethyl ammonium chloride was added to separate samples of a heating oil containing a polymeric dispersant additive after the formation of haze in the oil in the Waring Blender. The results of these tests are summarized in Table V and it can be seen that the addition of the chloride after haze formation had no effect whatsoever.

Table V

#### EFFECT OF ADDITION OF DICOCO DIMETHYL AMMONIUM CHLORIDE TO FUELS CONTAINING WATER-HAZE

|    | Fuel                                                                                                                               | Waring Blender haze test, percent light transmission after 6 hrs. |
|----|------------------------------------------------------------------------------------------------------------------------------------|-------------------------------------------------------------------|
| 10 | Base heating oil+0.01% polymeric dispersant B <sup>1</sup>                                                                         | 4                                                                 |
|    | Base heating oil+0.01% polymeric dispersant B <sup>1</sup> +0.0005% dicoco dimethyl ammonium chloride added after haze formation   | 4                                                                 |
| 15 | Base heating oil+0.005% polymeric dispersant B <sup>1</sup>                                                                        | 5                                                                 |
|    | Base heating oil+0.005% polymeric dispersant B <sup>1</sup> +0.00075% dicoco dimethyl ammonium chloride added after haze formation | 5                                                                 |

<sup>1</sup> Polymeric dispersant B was a mixture of 8 parts of a C<sub>12</sub> tertiary alkyl primary amine and 1 part of a copolymer prepared from 8 parts of Lorol methacrylate and 2 parts of beta diethylaminoethyl methacrylate.

#### EXAMPLE 6

In order to further test the effectiveness of dicoco dimethyl ammonium chloride, full-scale tanker tests were carried out by transporting 140,000 barrels of heating oil containing 0.005 wt. percent of a polymeric stabilizing additive in an ocean-going tanker from the Gulf coast to a New Jersey port. The additive employed was a mixture of 8 parts of a C<sub>12</sub> tertiary alkyl primary amine and 1 part of a copolymer prepared from 8 parts of Lorol methacrylate and 2 parts of beta diethylaminoethyl methacrylate. About 80,000 barrels of the oil contained 0.0005 wt. percent of dicoco dimethyl ammonium chloride. This oil was transported in 7 tanks of the ship. The remaining 60,000 barrels of oil was free of haze inhibitor and was transported in 12 tanks of the ship. There was about 4 inches of water in the bottom of each tank.

Upon completion of the voyage, the oil containing the dicoco dimethyl ammonium chloride and the oil free of the inhibitor were pumped into separate shore tanks of 112,000 barrels capacity. Hourly haze readings (percent haze equals 100—percent + transmission relative to fuel filtered bright) were made during the pumping at (1) the line on the dock (2) the line on the shore, and (3) the receiving tank. Haze readings on the line at the dock showed initial values of 80 to 90% with and without the ammonium chloride. The haze thereafter leveled off during pumping at from 45 to 50% in the oil which did not contain the additive of the invention; whereas haze in the oil containing the additive leveled off at from 7 to 8%. The other haze readings showed similar advantages for the additive.

After completion of the pumping described above, settling of the haze in the two shore tanks was observed at intervals for several days. The results of these observations are shown in the attached drawing. As can be seen from the drawing, the oil containing the dicoco dimethyl ammonium chloride had settled to 10% haze in 20 hours and contained only 1% haze after 62 hours. After 64 hours the oil without the additive had leveled off at 11% haze.

#### EXAMPLE 7

A turbo-jet engine fuel boiling between 275° F. and 480° F. contains 0.02 wt. percent of a copolymer of 50 parts of decyl methacrylate, 30 parts of octadecyl styrene and 20 parts of 4-vinyl pyridine as a polymeric dispersant stabilizing additive. The water tolerance properties of this fuel are improved by the addition of 0.002 wt. percent of didodecyl dimethyl ammonium chloride.

#### EXAMPLE 8

A diesel fuel is stabilized by the incorporation therein of 0.01 wt. percent of a copolymer of 80 parts of lauryl acrylate and 20 parts of beta methylamino butyl vinyl ether and 0.08 wt. percent of a mixture of tertiary alkyl

primary amines derived from  $C_{18}$  to  $C_{21}$  polypropylene. To this fuel is added 0.008 wt. percent of dodecyl tetra-decyl dimethyl ammonium chloride in order to improve its water tolerance.

The preceding examples illustrate the effect of dicoco dimethyl ammonium chloride and closely related compounds upon the formation of persistent haze and stable emulsions in hydrocarbon oils. The dialkyl dimethyl ammonium chlorides having alkyl groups consisting of at least 50%  $C_{12}$  to  $C_{14}$  radicals reduce both haze formation and emulsification even though water extracted; whereas other closely related compounds are ineffective to reduce haze, have no effect upon emulsification, or are almost completely extracted from the oil by small amounts of water. A wide variety of commercial demulsifiers, many of which are believed to be imidazolium compounds and other quaternary ammonium salts, have no beneficial effect upon haze formation and emulsification in the presence of polymeric dispersant stabilizing additives or actually increase haze formation in such oils. This singular effectiveness of the additives of the invention permits a significant improvement in the properties of petroleum products, simplifies the handling and storage of such products, and increases their marketability.

What is claimed is:

1. A petroleum distillate fuel boiling in the range between about 75° F. and about 750° F., having incorporated therein from about 0.001 wt. percent to about 1.0 wt. percent of an ashless oil-soluble polymeric dispersant stabilizing additive selected from the group consisting of (a) a copolymer of an alkyl chloropropylene-oxy mixed ester of an unsaturated conjugated dibasic acid and a polymerizable organic monomer containing a vinyl group and (b) a nitrogen-containing addition-type copolymer of an amine-free monomer containing one polymerizable ethylene linkage and an aliphatic hydrocarbon chain of from 8 to 18 carbon atoms with a monomer containing a nitrogen atom and one polymerizable ethylene linkage, and from about 0.00025 wt. percent to about 0.01 wt. percent of a dialkyl dimethyl ammonium chloride in 40 which at least 50% of the alkyl groups are  $C_{12}$  to  $C_{14}$  radicals.

2. A fuel as defined in claim 1 wherein the concentration of said dialkyl dimethyl ammonium chloride ranges from about 0.0005 wt. percent to about 0.001 wt. percent. 45

3. A fuel as defined in claim 1 wherein said dialkyl dimethyl ammonium chloride is didodecyl dimethyl ammonium chloride.

4. A fuel as defined in claim 1 wherein said dialkyl dimethyl ammonium chloride is technical dilauryl dimethyl ammonium chloride.

5. A fuel as defined in claim 1 wherein the concentration of said polymeric dispersant ranges from about 0.001 wt. percent to about 0.05 wt. percent.

6. A fuel as defined in claim 1 containing a tertiary alkyl primary amine having from 8 to 18 carbon atoms per molecule in a concentration of from about 2 to about 18 times the concentration of said copolymer.

7. A fuel as defined in claim 1 wherein the polymerizable organic monomer is a vinyl ester of a short chain fatty acid.

8. A fuel as defined in claim 1 wherein the polymerizable organic monomer is a mixture of an alkyl fumarate and a vinyl ester of a short chain fatty acid.

9. A petroleum distillate fuel boiling in the range between about 75° F. and about 750° F. containing about 0.001 to about 1.0 wt. percent of a copolymer of an acrylic acid ester of a  $C_{10}$  to  $C_{18}$  saturated aliphatic alcohol and a tertiary amino alkyl acrylate and from about 0.00025 wt. percent to about 0.01 wt. percent of dicoco dimethyl ammonium chloride.

10. A petroleum distillate fuel boiling in the range between about 75° F. and about 750° F. containing from about 0.001 wt. percent to about 1.0 wt. percent of a copolymer of from about 2 to about 1/20 parts of isoctyl chloropropyleneoxy maleate and 1 part of a mixture of vinyl acetate and tallow fumarate and from about 0.00025 wt. percent to about 0.01 wt. percent of dicoco dimethyl ammonium chloride.

11. A petroleum distillate fuel boiling in the range between about 75° F. and about 750° F. and containing from about 0.00025 wt. percent to about 0.01 wt. percent of dicoco dimethyl ammonium chloride and from about 0.001 wt. percent to about 1.0 wt. percent of a copolymer of a  $C_{10}$  to  $C_{18}$  primary alcohol ester of methacrylic acid and beta diethylaminoethyl methacrylate.

12. A fuel as defined in claim 11 to which has also been added from about 0.003 wt. percent to about 0.8 wt. percent of a  $C_{12}$  tertiary alkyl primary amine.

#### References Cited in the file of this patent

#### UNITED STATES PATENTS

|           |                |       |                |
|-----------|----------------|-------|----------------|
| 2,550,982 | Eberz          | ----- | May 1, 1951    |
| 2,737,452 | Catlin et al.  | ----- | Mar. 6, 1956   |
| 2,805,925 | Biswell        | ----- | Sept. 10, 1957 |
| 2,861,874 | O'Kelly et al. | ----- | Nov. 25, 1958  |

#### OTHER REFERENCES

"Surface Active Agents and Detergents," by Schwartz et al., vol. II, copyright 1958, p. 197.